

## UNITED STATES PATENT OFFICE.

ELWOOD EBIE AND GEORGE A. RICHTER, OF BERLIN, NEW HAMPSHIRE, ASSIGNEES TO  
BROWN COMPANY, OF BERLIN, NEW HAMPSHIRE, A CORPORATION OF MAINE.

## PROCESS OF BLEACHING CELLULOSIC MATERIAL.

No Drawing.

Application filed November 17, 1921. Serial No. 515,899.

*To all whom it may concern:*

Be it known that we, ELWOOD EBIE and GEORGE A. RICHTER, both citizens of the United States, residing at Berlin, in the county of Coos and State of New Hampshire, have invented new and useful Improvements in Processes of Bleaching Cellulosic Material, of which the following is a specification.

10 The object of the present invention is to provide a method for super-bleaching bleached cellulosic pulp by which such bleached pulp may be further bleached and whitened to an extent not heretofore possible, all without loss in strength and without affecting other desirable characteristics of the material.

While we shall describe a process embodying our invention as practiced in connection with sulphite pulp, it will be understood that the process may be practiced with other forms of cellulosic materials if desired.

Ordinarily paper pulp or cellulosic pulp is bleached by the use of an alkaline hypochlorite solution, and, in carrying on this operation, it is necessary either to sacrifice strength and other desirable qualities of the pulp to attain a desired degree of whiteness, or else to sacrifice the whiteness of the stock in order to preserve the strength and other desirable qualities in the pulp. As indicating more particularly what we have in mind as the other desirable characteristics of the cellulosic material, particularly of sulphite pulp for example, it is known that the bleaching operation affects the proportion in which cellulose of the order of alpha, beta and gamma cellulose are found in the finished stock. An excess of beta cellulose in the stock results in a loss in strength of paper produced from the stock, and this is likewise true of paper formed of stock in which there is an excess of gamma cellulose. On the other hand, however, it is desirable that the stock should contain a certain proportion of beta cellulose and possibly gamma cellulose, as, since alpha or resistant cellulose is hydrated with more difficulty than either beta or gamma cellulose, the presence 50 of certain proportions of beta and possibly

gamma cellulose in the stock makes possible the hydration of the entire stock during the beating operation in a shorter time and with greater ease than if the stock consisted solely of alpha cellulose. The degree of shrinkage of a sheet of paper during drying, formed of a given stock, is dependent upon the proportions of the beta and gamma cellulose to the alpha cellulose in the initial stock, since the shrinkage increases with the increase in proportion of beta and gamma cellulose, so that it is desirable that there should not be excessive quantities of the latter forms of cellulose in the bleached stock. Over, or excess 55 bleaching unduly increases the proportions in the finished product of these two forms of cellulose.

For indicating more or less roughly the proportions of alpha cellulose to beta and gamma cellulose in the bleached stock, it is customary to ascertain the copper number of such stock. Speaking generally, the copper number represents a semi-quantitative measure of oxidation products resulting 60 from the action of the bleach or other oxidants on sulphite pulp. The more severe the bleaching action, the higher is the final copper number due to the increased proportion 65 of those constituents responding to the beta and gamma cellulose determination. A normally bleached sulphite pulp shows a copper number of approximately 3 to 3.5. An increased copper number in the sulphite pulp is indicative of a high percentage of shrinkage during drying of the stock, a high color, 70 low strength and excessive "slowness" of the stock when beaten. Thus it will be seen that in the bleaching of pulp, if the bleaching reaction be carried on to a point where a very 75 white color in the final product is secured, there are losses in other qualities which are necessary or desirable for the production of a fine paper; and, on the other hand, where the bleaching reaction is stopped to preserve 80 the desirable characteristics of the stock, the stock itself has not obtained its highest degree of whiteness. The color of bleached 85 pulp is measured by a colorimeter, the variations in color, according to given standards, 90 95 100

being designated arbitrarily by numbers in a certain order of progression from 90 to 105. A normally well bleached pulp, possessing the desirable characteristics of strength, etc., 5 shows a color of about 99, which corresponds to the majority of bleached sulphite fiber commercially on the market.

We have discovered that it is possible to produce what may be termed a super-bleached pulp, having a high degree of whiteness without loss of or injury to the other desirable qualities and characteristics of cellulosic materials, by subjecting pulp (bleached in the ordinary way as by the use 10 of an alkaline hypochlorite) to the action of chlorine, either free or in solution in water. Our process, therefore, involves two stages, namely that of bleaching the stock in the ordinary way until a product is produced 15 showing a color of from say 95 to 99, and then super-bleaching it by subjecting the bleached stock to the action of chlorine in order to remove the remaining traces of ligneous or other coloring matter. A 20 stock, bleached to a point where it shows a color number of 95 to 99, tests high in strength, has a relatively low coefficient of shrinkage in drying, a high percentage of alpha cellulose and relatively low percent- 25 age of alpha cellulose and relatively low percentages of beta and gamma cellulose, assuming, of course, that the stock has not been injured in the initial liberation of the fiber by the process of digestion. By treat- 30 ing such a stock with a small quantity of chlorine under proper temperature conditions and for a limited period of time, the stock may be super-bleached and whitened to a point where it shows practically no traces 35 of color with practically no diminution in strength and with but slight variations in the relative proportions of the alpha, beta, and gamma cellulose.

In carrying on the first stage of the process by which bleached pulp is produced, the initial unbleached fiber is, by the use of the usual apparatus (e. g., pulp thickeners), brought to a stock concentration varying from 3% to 17%, this concentration depending 40 upon the particular apparatus which is subsequently used for bleaching. Ordinarily a calcium hypochlorite solution, containing about 32 grams of available chlorine per liter, is added to the stock in sufficient quantity to correspond to from 10% to 25% of bleach powder based on the quantity of dry pulp stock. The mixture is maintained in agitation for a sufficient time to allow complete reaction, after which the stock is 45 washed free of the reaction products, a small amount of antichlor being added when necessary to remove the remaining traces of the chlorine products. To prevent too rapid an oxidation of the lignin content, the temperature is regulated, since a temperature

above 100° F. usually causes the formation of oxycellulose and thereby affects the strength of the finished bleached stock. The bleached stock, which is thus produced, represents the ordinary commercial bleached pulp having a color number of approximately 97 to 99, a copper number of about 2.9 to 3.5 with a strength of 120 expressed in arbitrary units. This bleached stock is now subjected to the second stage of the process, 50 namely to the action of the chlorine by which it is super-bleached. As previously stated, the chlorine may be used either as a gas which is brought into contact with the wet stock, or it may be used as an aqueous chlorine solution which is added to the wet stock in sufficient quantities to give the desired result. These two ways of introducing the chlorine into the stock give substantially similar results. In practice, it is usually easier to control the amount of the chlorine employed for a given quantity of pulp by forming it into a solution. Where gaseous chlorine is employed, it may be either concentrated or it may be diluted 55 with air. By the addition of chlorine equivalent to from 0.2% to 0.5% by weight of the original air-dried stock, we are able to increase the color number to 102 to 103 without sacrificing in any way the strength and other desirable qualities of the finished stock. The reaction usually takes from 15 to 20 minutes. The pulp, as a result of the treatment, assumes a very pale yellowish tint, doubtless due to the soluble reaction 60 products resulting from the treatment. A bisulphite solution is then added to the pulp in sufficient quantities to neutralize any resulting hydrochloric acid and to combine with any remaining traces of chlorine. The bisulphite may be added either in the form of sodium or calcium and usually contains an excess of free sulphurous acid. The stock, of course, is agitated, and, after the addition of the bisulphite, sufficient time is 65 allowed to elapse for effecting a complete mixture, and the stock is then thoroughly washed with clean water and is ready for screening, riffling and other subsequent operations. It is not necessary that the stock should be washed at the end of the first stage of operations in carrying out our process, as the pulp may be treated with chlorine before the washing takes place. A saving of 70 chlorine and a somewhat higher color is obtained, however, if the stock is washed at the end of the first stage of operations before the chlorine is added. Instead of subjecting the stock in the second stage of the operations to a single acid treatment, it is quite evident that the stock may be first treated with chlorine, then washed, then given a second treatment of chlorine, followed by a final washing, the addition of the sulphite for neutralization of the hydro- 75 80 85 90 95 100 105 110 115 120 125 130

chloric acid and for reaction with the remaining traces of chlorine being omitted after the first treatment with chlorine.

As indicating results which have been obtained by the treatment with chlorine of a bleached pulp resulting from the first stage of operations, we present a table showing the effect of .5% chlorine based on 100% pulp by weight for 20 minutes at 10 room temperature on a 10% stock suspension in water. The figures in the first column represent the characteristics of the bleached pulp after the first stage in the bleaching operation and the second column 15 shows the tests of the same pulp after being subjected to the chlorine treatment.

| 20                               | Test. | Bleached pulp, first stage. | Super-bleached pulp, second stage. |
|----------------------------------|-------|-----------------------------|------------------------------------|
| Strength.....                    |       | 120                         | 120                                |
| Slowness.....                    |       | 10' 35"                     | 9' 20"                             |
| Shrinkage.....                   |       | 20.8                        | 20.2                               |
| 25 Per cent alpha cellulose..... |       | 87.7                        | 89.5                               |
| Per cent beta cellulose.....     |       | 2.1                         | 2.2                                |
| Per cent gamma cellulose.....    |       | 10.2                        | 8.3                                |
| Per cent total cellulose.....    |       | 98.92                       | 99.42                              |
| Copper number.....               |       | 2.95                        | 3.25                               |
| Color.....                       |       | 99                          | 101+                               |

30 We have stated that we may introduce gaseous chlorine into the aqueous pulp or may add to the pulp an aqueous chlorine solution. In each case, the chlorine, of course, goes largely into solution in water with the probable formation of some hypochlorous acid (HOCl), so that undoubtedly a portion of the lignin content remaining in the stock is oxidized. On the other hand, however, there is a perceptible yellowish tint in the stock after the treatment which would indicate that a chlorination of certain of the stock constituents had taken place, so that in all likelihood there is an action of the free chlorine directly on the stock in addition to the oxidation resulting from the presence of the hypochlorous acid.

40 We are aware that it has been proposed primarily to bleach unbleached pulp with a chlorine solution in which the resulting hypochloric acid is neutralized by a base such as sodium or calcium carbonate. The action of such a bleaching solution, however, upon unbleached stock is exceedingly harsh or else an excess quantity of the base must be employed. In any case, however, such a treatment will not give a stock having the 45 exceptional color produced by the process herein described without destroying or injuring the strength and other desirable characteristics of the stock.

50 60 What we claim is:

1. The herein described process of super-bleaching cellulosic material, which comprises two stages of operations, namely, subjecting the unbleached material to the action of an alkaline bleaching agent

to bleach and whiten said material without markedly decreasing the strength thereof, washing said material and removing the reaction products, and then subjecting such material to the action of chlorine 70 whereby the said material is super-bleached to a greater whiteness without substantially decreasing the strength or materially affecting the other characteristics of such 75 cellulosic material.

2. The herein described process of bleaching cellulosic material, which comprises two stages of operations, namely, first subjecting the unbleached material to the usual bleaching action of an alkaline hypochlorite 80 to initially bleach the same, and removing the products of reaction, and second, subjecting the bleached material to the action of chlorine to increase the whiteness of said material without any substantial change in 85 the strength or beating qualities thereof.

3. A process of super-bleaching bleached cellulosic material, which comprises subjecting said bleached material to the action 90 of chlorine to increase the whiteness of said material without any substantial change in the strength or beating qualities of the material.

4. A process of super-bleaching bleached cellulosic material, comprising the steps of removing the reaction products from the first bleaching operation, and then treating the material with chlorine to super-bleach the bleached material without substantial 100 change in the strength or beating qualities of the material.

5. The herein described process of bleaching cellulosic material, which comprises the following stages of operations, 105 namely, subjecting the unbleached material to the bleaching action of an alkaline hypochlorite to initially bleach the same as ordinarily, washing the material to free it of the bleaching agent and the products of the reaction, and treating the bleached pulp with an aqueous solution of chlorine with the chlorine in the proportion of about 0.2% to 0.5% by weight of the original air-dried cellulosic material to super-bleach the 110 bleached material.

6. The herein described process of super-bleaching cellulosic pulp which comprises the following operations, namely, first, producing a bleached pulp by subjecting the unbleached material to the bleaching action 120 of an alkaline hypochlorite to initially bleach the same and washing the material to free it of the bleaching agent and the products of the reaction, and, second, super-bleaching the bleached pulp by treating it with an aqueous solution of chlorine, with the chlorine in the proportion of about 0.2% to 0.5% by weight of the original air-dried cellulosic material, adding an antichlor 125 to the mixture and finally washing such

mixture to free the cellulosic material from impurities.

7. A super-bleached cellulosic pulp product containing approximately 89% alpha cellulose and approximately 2% beta cellulose and having approximately the same strength and beating qualities as the same pulp when

subjected to the ordinary commercial bleaching operation, but having an increased whiteness over said last mentioned pulp.

In testimony whereof we have affixed our signatures.

ELWOOD EBIE.  
GEORGE A. RICHTER.